

# UNITED STATES PATENT OFFICE.

SILAS R. DIVINE, OF LOCH SHELDRAKE, NEW YORK, ASSIGNOR TO THE  
REND ROCK POWDER COMPANY, OF NEW JERSEY.

## EXPLOSIVE COMPOUND

SPECIFICATION forming part of Letters Patent No. 289,759, dated December 4, 1883.  
Application filed July 23, 1883. (No specimens.)

*To all whom it may concern:*

Be it known that I, SILAS R. DIVINE, of  
Loch Sheldrake, Sullivan county, State of New  
York, and a citizen of the United States, have  
5 invented an Improved Explosive Compound,  
of which the following is a full, clear, and ex-  
act specification.

My invention consists in an explosive com-  
10 pound for use, chiefly, in blasting, composed of  
a solid ingredient—such as chlorate of potash—  
and a liquid ingredient consisting of a mixture  
of “dead-oil” and nitro-glycerine, which in-  
gredients are in themselves non-explosive by  
15 percussion, and hence may be with safety  
handled and transported separately, and which  
may be combined to form the explosive by  
allowing the solid to absorb the liquid ingre-  
dient, substantially in the proportions and as  
20 and for the purpose set forth.

The object of my invention is to produce a  
25 compound which is susceptible to explosion,  
and one the strength or explosive force of  
which may be graded or regulated at pleasure.

The solid ingredient of my compound con-  
25 sists, preferably, of crushed or powdered chlo-  
rate of potash, although perchlorate or per-  
manganate of potash may be thus employed.  
The liquid ingredient of my compound I com-  
pose of preferably two parts of dead-oil to one  
30 part of nitro-glycerine, as these proportions  
constitute a mixture which is capable of being  
handled and transported safely, and which at  
the same time, when combined with the solid  
ingredient, in the proportions named, unite  
35 most effectively therewith to form an explo-  
sive. The theoretical proportions in which the  
chlorate of potash and the said mixture com-  
bine most effectively, as stated, are about five  
parts of the chlorate of potash to one part of  
40 the mixture; but for the purpose of somewhat  
decreasing the sensitiveness of the compound

in its practical use, it is found desirable to  
sometimes decrease the said proportions to  
about four parts of the chlorate of potash to  
one of the mixture. The exact theoretical pro-  
portions may therefore be varied from and  
still an efficient explosive be produced. 45

The proportions of the dead-oil and the  
nitro-glycerine which are indicated as pref-  
erable in the mixture constituting the liquid  
ingredient may be varied somewhat; but it is  
not desirable that the nitro-glycerine in the  
mixture should be decreased below about  
20 twenty per cent., as its effect in the compound  
thereby apparently disappears, while it is not  
desirable that it should be increased above fifty  
or sixty per cent., as its “sensitizing” effect  
is then too greatly augmented for the purposes  
of this invention. 55

Other fluid hydrocarbons than dead-oil 60  
which are practically non-volatile in a free  
state at ordinary temperatures, and which are  
solvents of nitro-glycerine, or such nitro com-  
pounds as nitro-benzole, may be used with the  
nitro-glycerine to form the described mixture 65  
constituting the liquid ingredient of the com-  
pound.

What I claim as my invention, and desire to  
secure by Letters Patent, is—

The herein-described explosive compound, 70  
composed of chlorate of potash, constituting  
the solid ingredient, and dead-oil and nitro-  
glycerine, substantially in the proportions set  
forth, constituting the liquid ingredient, the  
said solid and liquid ingredients being me-  
chanically united, substantially in the propor-  
tions and as and for the purpose specified. 75

SILAS R. DIVINE.

Witnesses:

A. G. N. VERMILYA,  
A. S. FITCH.